

## UNITED STATES PATENT OFFICE

2,083,275

## MANUFACTURE OF SILICON STEEL SHEETS

Orlando E. Romig, Gary, Ind., assignor to American Sheet and Tin Plate Company, a corporation of New Jersey

No Drawing. Application August 29, 1930, Serial No. 478,798

## 1 Claim. (Cl. 148—12)

This invention relates to the manufacture of silicon steel products and although not limited thereto, more particularly relates to the manufacture of silicon steel sheets or sheet material and plates.

Certain parts of electrical apparatus, having alternating magnetic fields, such as transformer cores, armature cores, pole pieces and magnetic poles of various kinds are preferably or necessarily of a laminated structure, being composed of plates or laminations stamped or cut from sheet iron or steel. All sheet metal for such analogous purposes should possess a high degree of magnetic permeability, a high degree of electrical resistivity in order to minimize eddy current losses, a low degree of magnetic hysteresis, and be physically strong and as pliable as possible and free from brittleness. Some sheet iron and steel, notably that employed in transformer cores and to a lesser extent, that used in alternating current generators, must be characterized by low hysteresis loss. In transformer cores especially the hysteresis loss is a most important consideration; but it is desirable to combine low hysteresis loss with high permeability and the physical properties hereinbefore mentioned.

It is common knowledge that steel containing the element silicon in sufficient amounts but otherwise about as free as is commercially practicable from all other elements except iron, furnishes, if properly processed, a sheet which meets all the above described requisites to a remarkable degree. Transformer sheets must also be non-aging, that is, they should not deteriorate with age, especially as regards to hysteresis losses. These electrical properties of silicon sheets as to eddy current losses and hysteresis losses are commonly tested in an Epstein apparatus, the combined losses being measured at various inductions. Most manufacturers of silicon steel sheets, therefore, sell their sheets guaranteeing them to test on an average below a certain maximum core loss expressed watts per pound or watts per kilogram at a certain induction and a given frequency as agreed between the manufacturer and purchaser.

For every ingot of ordinary steel a sheet of certain maximum physical excellence or quality of finish may be obtained, depending on its nature and chemical composition. Similarly, a certain minimum of hysteresis loss is possible for the sheets rolled from an ingot of silicon steel. The degree of excellence of the sheets depends considerably on the treatment which is

given the sheets in hot rolling, pickling, cold rolling and heat treating.

According to the well known laws of metallurgy and metallography, all steel, including silicon steel, is known to be made up of crystals or grains which are of various sizes and shapes, depending on the treatment accorded the steel in processing.

It is also well known that when dealing with certain types of low carbon steels the crystals or grains can be made to grow and absorb the neighboring grains, thus increasing the crystal or grain size in the steel considerably. This crystal growth is brought about by straining the crystals to a certain point and following this straining with an annealing operation which allows the crystals to coalesce and grow.

These large grains are usually undesirable in most steel where good ductility and considerable strength is desired but in the case of silicon steels used for electrical apparatus it is generally accepted that large grains tend to lower the hysteresis losses of the steel. The use of silicon in electrical steel tends to increase the crystal or grain size of the steel and this is one of several reasons why silicon is useful in electrical steels.

However, by using the ordinary rolling and annealing processes, the size of the crystals or grains obtainable in silicon sheets is somewhat limited. By certain special hot rolling practices it has been found that large grains can be produced after a subsequent annealing operation. However, this variation in hot rolling practice is fairly sensitive, requires an additional heating and careful manipulation of hot packs. This practice, when successfully manipulated, tends to produce increased grain size in silicon sheets with attending low hysteresis losses. These hot rolling processes are good and very satisfactory results have been obtained by them.

The present invention has eliminated the necessity of using these special hot rolling practices and provides a process or method of treating the silicon sheets or sheet material uniformly and successfully after they have been hot rolled without the variations in practice sometimes unavoidable in handling hot packs in hot rolling.

I have found that I can, by means of my process, induce in a heat treated silicon sheet exactly the degree of strain necessary to produce grain growth in the annealing of silicon sheets and with it the attendant superiority as to low hysteresis losses.

By my invention I am enabled to produce silicon

steel of much lower hysteresis loss than is possible by the usual mill practice in processing silicon sheets, the improvement due to our invention being quite definite and well marked and amounting to as much as 12 to 15 per cent. over sheets produced by the usual practice.

Moreover, my improved process enables me to treat sheets which have been brought to the minimum hysteresis loss possible under the usual methods of sheet rolling and to effect in them the marked improvement of hysteresis quality and this in addition to what little improvement is made in the eddy current loss due to reduction of gage.

15 In the usual methods of manufacturing silicon sheets, the sheets are produced under the usual hot mill practice of hot rolling sheets from bars, the hot rolled sheets are then cold rolled to flatten them, they are then pickled and heat treated or 20 box annealed. In practically all the prior art methods of manufacturing silicon sheets the sheets are cold rolled and box annealed although not all sheets are pickled or heat treated.

25 In carrying out my improved process the silicon steel bars are first hot rolled. They may be either "breakdowns" or finished hot rolled sheets or packs. If in packs, they may or may not be opened. The shearing or not shearing of the 30 packs, "breakdowns" or sheets is immaterial. They then may or may not be given the usual cold rolling pass to smooth out the bent opening corners or to flatten the sheet.

35 The sheets are then usually pickled if a scale-free surface is desired. This pickling step has little or no effect on the final product; therefore, the inclusion or elimination from the general process is immaterial.

40 The next step in this process, either before or after opening and followed by a flattening cold roll pass if desired, and after pickling sheets when desired, is to normalize the sheets by passing the sheets through a furnace which raises the sheets, 45 packs or "breakdowns" to a temperature of from 1500 to 2000 degrees Fahrenheit, more or less, this operation being most commonly done in a reducing atmosphere. I have found the above temperature range most effective but a lower or higher temperature may be used with good results.

50 The term "normalize" as commonly used in the steel making arts is used to indicate a heat-treatment consisting of heating the steel above its so called transformation point followed by cooling rather quickly in air or a reducing atmosphere. Silicon steel does not act the same in the normalizing operation as does ordinary steel. Whether 55 silicon steel is actually normalized by heating as above described is an open question among metallurgists.

60 In this specification and in the claims the term "normalize" is used to define a heat treatment at from 1500 to 2000 degrees Fahrenheit, more or less, which serves to relieve the hot rolling strains and prepare the steel for its subsequent elongation or stretching. This treatment is preferably 65 carried out in a so-called normalizing furnace but may also be carried out in other forms of heat treating furnaces.

70 The above normalizing step serves to eliminate a large part of the rolling strains and hardness induced by the hot and cold rolling operations.

75 However, all of the strains are not relieved by this normalizing step but the strain has been reduced in the sheets to somewhat below "critical strain" (that amount of tension or compression in a sheet or in a bar which will promote maxi-

mum grain growth when said material is subsequently annealed). Sheets with varying amounts of strain up to this point are all reduced to a common basis of strain. All of the sheets are therefore put into such a physical condition that a small amount of fairly easily controllable strain can be applied, thus bringing all the individual sheets to a point where they have been "critically strained" or more, which is necessary before further treatment to get the maximum improvement in their hysteresis losses.

5 The above normalizing step is not to be confused with ordinary annealing. Ordinary annealing produces a grain growth in silicon steel which is somewhat beneficial whereas this normalizing step, although not alone sufficient to produce the desired electrical properties is very much superior to an ordinary annealing at this stage of the process.

15 The normalizing step of this method destroys 20 the hot rolling grain structure in order to permit the following steps to develop a proper grain growth not possible unless the hot rolling grain structure is destroyed.

25 In order to introduce the strain necessary to 30 promote grain growth according to the natural laws governing the sciences of metallurgy and metallography the normalized sheets are elongated or stretched preferably in a cold rolling mill. This elongation or stretching produces the critically strained condition necessary for the promotion of uniformly large crystals or grains of silicon steel.

35 Experience has shown that an elongation of 1 to 2½ per cent. is preferable although I do not 40 wish to limit my invention to this range of elongation since quite satisfactory results have been obtained by more or less elongation. It will also be noted that I do not wish to limit myself to the use of cold rolling for producing the elongation 45 since other methods of stretching or elongating the sheets may be employed.

50 The sheets are preferably stretched or elongated while they are yet warm from the normalizing step and this is especially true when the 55 sheets contain from 2 to 5 per cent. silicon since such sheets are much more ductile and workable when warm and may be elongated with less danger of breakage. The temperature at which the sheets are best suited for elongation or stretching depends largely upon practical working conditions, as for instance, whether the weather is hot or cold, whether the sheets are brittle, the width and gage of the sheets and many other considerations.

55 The temperature at which the sheets are best suited for stretching or elongation, however is generally from 200 to 400 degrees Fahrenheit for 60 physical reasons before mentioned but I do not wish to limit myself to any specific temperature or range of temperatures as I have found that sheets stretched or elongated at other temperatures have worked satisfactorily.

65 In order to obtain the elongation most desirable I have found that it is generally most practical to put one to ten sheets through either a two-high, three-high or a four-high cold rolling mill, especially when the gage or thickness is slight, but I do not wish to limit myself to this 70 number of sheets nor to this method of elongating or stretching.

75 After stretching or elongating the sheets they generally are next subjected to box annealing in order to further develop the grain growth and produce sheets having a minimum hysteresis loss 75

and other excellent qualities desirable for transformer cores, alternating current generators, resistance grids, etc. In obtaining sheets by my method which have equivalent electrical properties of sheets produced by the prior arts, a reduction in silicon content is permissible, resulting in a more ductile product, since this reduction in silicon content more than compensates in ductility for the brittleness accompanying larger grain size. Sheets are therefore more workable when sheared or stamped into shapes.

The words "sheet" or "sheet material" used throughout this specification and claim are meant to include all sheet-like bodies whether in sheet or strip form, plate, packs or "breakdowns" and is to be so construed.

It will also be noted that I do not wish to be limited to the exact temperatures at which the sheets are preferably stretched or elongated after normalizing, since this step may be carried out with good results at any temperature below the critical or recalescence point.

While I have described a certain specific sequence of steps and certain specific details of the several steps it will be understood that I do not wish to be limited thereto since various modi-

fications may be practiced without departing from the scope of my invention, as defined in the appended claim.

I do not wish to limit myself to any specific annealing temperature or range of temperature as satisfactory results have been obtained with extreme variations in temperature, depending upon the nature of the steel, the percentage of silicon therein, the amount of strain in the sheets and the iron loss desired.

I claim:

The method of preparing silicon steel sheet material for electrical purposes which includes hot rolling the sheet material, normalizing the sheet material to reduce the strains resulting from hot rolling to a point somewhat below the point of critical strain, stretching and elongating the normalized sheet material while still materially above atmospheric temperature from the normalizing operation to introduce the critical strain necessary for the promotion of uniformly large crystals or grains, and then annealing said stretched and elongated sheet material to induce the maximum grain growth and improve the electrical qualities thereof.

ORLANDO E. ROMIG.